

July 17, 1962

M. G. WHITFIELD ET AL

3,044,156

TEMPERATURE RESISTANT BODY

Filed June 23, 1954

*FIG.1.*



*FIG. 2.*



*FIG. 3.*



INVENTORS.  
MARSHALL G. WHITFIELD  
AND VICTOR SHESHUNOFF  
BY

*Allen & Allen*

ATTORNEYS.

# United States Patent Office

3,044,156

Patented July 17, 1962

1

3,044,156

## TEMPERATURE RESISTANT BODY

Marshall G. Whifford, 2 Harvard St., Garden City, N.Y.,  
and Victor Sheshunoff, P.O. Box 702, Magnolia, Ark.

Filed June 23, 1954, Ser. No. 438,652  
7 Claims. (Cl. 29—194)

The present invention relates to improved metal bodies constituted of tungsten or molybdenum and ferrous alloys thereof, and more particularly to metal bodies containing substantial percentages of tungsten and molybdenum protected against deterioration in oxidizing atmospheres at high operating temperatures.

This is a continuation-in-part of our copending application, Serial No. 673,880, filed June 1, 1946, and entitled "Oxidation Protected Tungsten and Molybdenum Bodies and Method of Producing Same," which has now matured into Patent 2,682,101, dated June 29, 1954.

At the present time there are various industrial developments where alloys of special character are necessary, capable of retaining their high mechanical strength at high operating temperatures. Examples of such applications are particularly parts for jet engines and gas turbines in which the demands made on the structural parts with respect to their strength at elevated operating temperatures are extremely exacting.

Materials now employed for these purposes generally comprise alloys of iron and of nickel, in many cases with additions of cobalt, chromium, tungsten and molybdenum. Even the alloys of tungsten and molybdenum, while theoretically promising, proved very disappointing in actual practice. In general, few, if any, of these alloys had a useful life over 300 hours, necessitating frequent replacement of critically important structural elements at great trouble and expense.

As is known, tungsten and molybdenum are unstable when heated in air or in any other oxidizing atmosphere at temperatures in the range of 800° C., or above. The oxides formed on the surface of the tungsten and molybdenum bodies under such conditions sublime or boil away continuously to such a pronounced degree that these metals can only be used in a pure reducing atmosphere of hydrogen, or of an inert gas, such as argon, or in vacuum. The same difficulty is present with respect to alloys containing more than 15% of tungsten and molybdenum. Of course, this circumstance greatly restricted or even negated the usefulness of such metal bodies and, as a matter of fact, those skilled in the art strongly advised against the use of alloys containing tungsten and molybdenum in excess of 15% for high temperature applications. Although the outstanding problem was well known in the art and from time to time various suggestions and proposals were made to provide a solution therefor, none, as far as we are aware, of these suggestions and proposals was completely satisfactory and successful on a practical and industrial scale.

We have found that the problem may be solved in a remarkably simple and unique manner.

It is another object of the invention to provide a novel and improved method of preventing the surface sublimation and resulting deterioration of metal bodies constituted of tungsten, molybdenum, and alloys thereof when exposed to oxidizing atmospheres at elevated temperatures in the range of 800° C. and thereover.

It is a further object of the invention to provide a protective layer on the surface of tungsten and molybdenum bodies, said protective layer being essentially composed of an aluminum containing material.

It is also within the contemplation of the invention to provide a novel method of protecting tungsten and molybdenum bodies against surface sublimation at high operating temperatures while exposed to oxidizing

2

atmospheres which is simple in character and which may readily carried out on a practical and industrial scale at low cost.

The invention also contemplates a new article of manufacture in the form of a refractory metal body protected from oxidic surface deterioration comprising a core of tungsten or molybdenum, or alloys thereof with each other or with other metals, and a protective layer coated on said core.

Another object of the invention is the provision of means for avoiding the deterioration of protected bodies made of or containing molybdenum or tungsten or both due to excessive differences in coefficients of expansion as between the body and the coating.

Another object of the invention is the provision of coated bodies of the general class herein referred to in which beryllium is a constituent of the body or the coating or both.

Other and further objects and advantages of the invention will become apparent from the following description, taken in conjunction with the accompanying drawing, in which:

FIG. 1 is a fragmentary sectional view of a metal body embodying the principles of the invention during the process of its manufacture.

FIG. 2 is a similar view of an oxidation protected tungsten or molybdenum body having a bonding layer of nickel and a protective layer applied thereto, and

FIG. 3 is a longitudinal sectional view of a refractory metal body comprising a core of tungsten or molybdenum and having a partially diffused protective layer thereon constituted of an alloy of protective elements and molybdenum or tungsten.

Broadly stated, according to the principles of the invention, the tungsten or molybdenum bodies to be protected are coated preferably with a aluminum base material which may be pure aluminum or alloys rich in aluminum. This coating may be carried out by various procedures but best results are obtained by a hot dip method in which the metal bodies to be protected are immersed in a bath of molten metal for a predetermined length of time sufficient to provide a coating of the metal thereon. We have found that by this method there is formed a thin protective layer on the surface of the tungsten or molybdenum body which layer is essentially constituted of an alloy of coating metal with the base metal. Experimental work with tungsten and molybdenum bodies treated in accordance with the invention has indicated that these materials do not exhibit their normal oxide forming characteristics even at temperatures approximating the boiling point of aluminum and in many cases even at temperatures as high as 2000° C.

The bath of molten aluminum base material may be composed of high purity aluminum, commercially pure aluminum and of aluminum alloys having a relatively high aluminum content. Examples of such aluminum alloys are alloys containing 5% to 15% by weight of at least one of the elements selected from the group consisting of iron, nickel, chromium, cobalt and beryllium, the balance being substantially all aluminum. In addition, various other aluminum base materials containing other and further constituents may be used.

If desired, the bodies to be treated with the bath of molten aluminum base material may be subjected to a preliminary cleaning by sandblasting, burnishing and similar mechanical procedures. In most cases, however, such preliminary cleaning is not necessary. For example, rolled molybdenum sheet may be subjected to treatment by the bath of aluminum base material without any preliminary cleaning.

The temperature of the bath of molten aluminum base material may be subject to considerable variations in

accordance with its composition. Thus, in the case of a bath of commercially pure aluminum, temperatures in the range of 700° to 800° C. provide satisfactory results.

The aluminum coating treatment may be carried out continuously or by means of a bath type process. Particularly in the case of a continuous process, the treatment in the molten bath of aluminum base material may vary from a few seconds to several minutes depending on the initial temperature of the bodies to be treated, on their thickness or mass and to some extent also on the operating temperature of the bath. The thickness of the coating of aluminum base material is not critical but may be in the order of 0.002" to 0.004".

Examination of wire and sheet samples of tungsten and molybdenum, which have been treated with aluminum and exposed to high temperatures in oxidizing atmospheres, indicates that a high melting compound of aluminum with the tungsten or molybdenum core has been formed and that this alloy is free from the weakness of either the tungsten or molybdenum with regard to oxidizing to form a compound of low boiling or sublimation point on the surface. For example, samples treated by the method of the invention have been heated to temperatures a hundred degrees C. above the normal boiling point of aluminum before the aluminum boiled away, indicating that the alloys of aluminum with tungsten or molybdenum have extremely high boiling or sublimation points. Likewise, it has been found that the presence of aluminum on the surface of these metals, will permit their use for applications requiring substantial strength at elevated temperatures. The method of the invention is applicable with equal or similar results also to alloys of at least one of the metals iron, nickel, cobalt with tungsten or molybdenum, or both, containing substantial quantities of tungsten or molybdenum, such as at least 15% by weight, and also to alloys of tungsten and molybdenum.

Preferably, the aluminum coated tungsten and molybdenum containing bodies are heat treated to assure the formation of a high melting compound of aluminum with the tungsten or molybdenum core and thereby to obtain a completely stable product. It is also possible, however, to omit such heat treatment and to rely on the diffusion of the aluminum coating into the refractory core during the actual operation at elevated temperatures. If heat treatment is resorted to, the heat treating temperature may be in the order of 1300° C., although it is not restricted to such temperature.

While the method of the invention provides excellent results in protecting and stabilizing tungsten and molybdenum bodies, when treating these metals with aluminum or its alloys, occasionally small spots or areas are found which are alloyed only with extreme difficulty. We have found that this difficulty may be completely avoided by electrodepositing a thin film or layer of nickel on the surface of the tungsten or molybdenum and diffusing or at least heating the nickel plated sections in a non-oxidizing or reducing atmosphere at approximately 1000° C. before treating the sections of tungsten or molybdenum with aluminum. This modification of the method of the invention provides in most cases more uniform protection or alloying of the aluminum with the base metals.

The thickness of the electrodeposited nickel layer is not critical and may be subjected to considerable variations. In this connection, it may be observed that diffusion of the nickel layer may be accomplished not only by heating under non-oxidizing conditions but also by heating in an oxidizing atmosphere provided that sufficient nickel is present. As a matter of fact, electroplating with nickel may be immediately followed by the aluminum coating treatment. In this case, diffusion of the nickel layer is accomplished by the heating effect of the bath of aluminum base material, and the bath at the same time provides the non-oxidizing or protective environment.

It has been found that nickel is not the only metal which

is capable of providing this additional protection, but that in general iron group metals such as nickel, iron, cobalt, chrominum and manganese will accomplish substantially the same result. Moreover, we have found that in many cases copper and silver plates may provide equal or similar results.

While the exact reason for the beneficial effect of the preliminary deposit of nickel or other iron group metal is not fully understood, it is believed that these metals form alloys with aluminum more quickly than do tungsten and molybdenum and that these electrodeposited films act as temporary protectors until the aluminum can form its alloy with the tungsten or molybdenum which have a tendency to oxidize even at relatively low temperatures, such as red heat.

Referring now to the drawing, in FIG. 1 there is shown a metal body embodying the principles of the invention which comprises a base or core 10 of tungsten or molybdenum. Upon both faces of the core there is provided a thin coating 11 of aluminum or aluminum base material constituting a protective layer for the core. Of course, in actual manufacture, layer 11 is initially a coating of aluminum containing some tungsten or molybdenum and is bonded to the core by an aluminum rich alloy of these refractory metals caused by partial diffusion of the aluminum into the core. In service, or in the final stage of manufacture, the excess aluminum is partly oxidized and partly diffused to produce the alloy surface layer which is referred to in the foregoing.

FIG. 2 illustrates an example of the modification of the invention in which the tungsten or molybdenum core 20 is first coated with a thin film of nickel or other iron base metal 21 and thereafter is exposed to the effect of a molten bath of aluminum base material, such as, for example, commercially pure aluminum, thereby forming a protective layer 22 on the exterior of the core. As a result of the interaction of the core material with that of the layers 21 and 22 during the heating and coating treatments and subsequent service operation, the metal body is converted into the one shown in FIG. 3 wherein the individual existence of layers 21 and 22 has practically disappeared, such layers being combined into a layer 23 which is composed of an alloy rich in aluminum and containing appreciable amounts of nickel and tungsten or molybdenum.

While in the drawing fragmentary sectional views of refractory metal strips are shown which are coated with a layer of aluminum base material on both faces thereof, in actual practice, the refractory metal bodies are provided with a protective layer of the described character throughout their entire surface, including their ends and edges. In this manner, the said metal bodies are fully protected from deterioration at elevated operating temperatures.

In order to facilitate understanding of the invention by those skilled in the art, the following illustrative examples may be given:

#### Example I

A molybdenum sheet 0.015" thick, mill finish, was immersed in a bath of molten commercially pure aluminum having a temperature of 720° C., for 6 minutes. After removal from the bath and cooling, the material was tested by heating it to 1400-1500° C. in an oxidizing atmosphere for 4 hours, without noting any appreciable deterioration.

#### Example II

A molybdenum sheet about 0.020" thick was cleaned and a light coating of nickel was electrodeposited thereon. The plated sheet was heated for a few minutes in a reducing atmosphere at approximately 1000° C. The sheet was cooled and then treated by immersing in a bath of molten commercially pure aluminum, having a temperature of 740° C., for 3 minutes.

Although the present invention has been described in

connection with a few preferred embodiments thereof, variations and modifications may be resorted by those skilled in the art without departing from the principles of the invention. Thus, as it has been indicated in the foregoing, the principles of the invention are not restricted to the treatment of tungsten and molybdenum bodies but may be applied with equal or similar results to metal bodies composed of alloys of tungsten and molybdenum with each other or with other metals. The advantages of the invention in the case of tungsten and molybdenum alloys are particularly accentuated when such alloys contain at least 15% by weight of tungsten or molybdenum, or tungsten and molybdenum combined.

The teachings hereinabove made and the examples hereinabove given, applying to the coating of tungsten or molybdenum bodies (as defined) with aluminum or aluminum alloys (as defined), apply as well to the use of the metals silicon and beryllium as constituents of the initial coating. One of the purposes of the present invention is to avoid extraordinary discrepancies between the coefficients of expansion of the base metal and the coating material. As compared with aluminum which has a high coefficient of expansion, tungsten and molybdenum bodies have relatively low coefficients of expansion.

It has hitherto been known that the alloying of relatively large quantities of silicon with aluminum will provide a metal composite having a relatively lower coefficient of expansion, and in particular a coefficient of expansion substantially closer to that of ferrous bodies. For such purposes, as much as from 25% to 30% or more of silicon has been alloyed with aluminum.

It has been found, however, that such very large quantities of silicon give an aluminum alloy material which is more difficult to use in molten form as a hot dipping medium, and also that the formation of an adequate bond between the alloy layer and ferrous base metals is rendered more difficult.

Beryllium is a metal which has a coefficient of expansion substantially less than half that of aluminum. We have found that beryllium may be alloyed with aluminum to provide alloys having coefficients of expansion much closer to that of ferrous bodies and tungsten and molybdenum bodies as herein defined. When beryllium is added to aluminum, it is readily possible to secure coating alloys having coefficients of expansion very much lower than that of aluminum alone, and in particular coefficients of expansion substantially corresponding with those of conventional ferrous bodies, with the beryllium within the ranges set forth above, namely from about 5% to about 15%, and up to about 50% of the alloy.

It is readily possible to employ beryllium along with silicon. For example, an alloy can be formed of aluminum containing about 5% to 15% of beryllium and 5% to 50% silicon, balance being aluminum.

Beryllium in substantial quantities thus is seen to be a valuable component of aluminum or aluminum alloys used for coating where the object is to attain in the coating a coefficient of expansion much more nearly corresponding to that of the base metal, whether the base metal is to be coated by hot dipping or by the casting of the aluminum alloy against it. Moreover, beryllium has a substantially lessened tendency to interfere with the formation of a strong bond between the aluminum alloy and the base metal upon which it is coated.

In the formation of tungsten or molybdenum bodies which are to withstand oxidative deterioration at the high temperatures mentioned herein, the beryllium does not interfere with the action hereinabove described. In fact, tungsten and molybdenum bodies, resistant to oxidative deterioration at high temperatures, can be produced by coating tungsten or molybdenum bodies (as defined) with beryllium alone, in spite of the high avidity of the last named metal for oxygen. The use of interface metal coatings as hereinabove disclosed between the

aluminum alloy and the base metal is equally effective with beryllium alone or with aluminum alloys containing beryllium or beryllium and silicon.

In the production of coated bodies having a minimum difference between the coefficients of expansion of the bodies and the coatings thereon, it is possible not only to diminish the coefficient of expansion of the coatings, but also to raise the coefficient of expansion of the bodies. Where tungsten and molybdenum bodies are spoken of above, not only are bodies of pure molybdenum or tungsten or mixtures of the two contemplated, but also ternary or complex alloys containing at least substantially 15% of tungsten or molybdenum or a mixture of the two. The coefficient of expansion of such ternary or complex alloys is higher than that of molybdenum or tungsten alone. But it is possible to raise the coefficient of expansion of such bodies by alloying the molybdenum or tungsten or ternary alloys containing them with such elements as chromium. This may ordinarily be done without sacrifice of desirable physical properties.

When coating tungsten or molybdenum or ferrous bodies with beryllium or aluminum alloys containing beryllium, a protective atmosphere will normally be maintained over the bath since beryllium is more subject to oxidation than aluminum.

Modifications may be made in the invention without departing from the spirit of it. The invention having been described in certain exemplary embodiments, what is claimed as new and desired to be protected by Letters Patent is:

1. A body formed from metal chosen from a class consisting of tungsten, molybdenum, mixtures of the two, and ferrous alloys containing at least 15% of any of the foregoing, hot coated with a bonded layer of aluminum containing substantially 5% to 50% beryllium.

2. A body formed from metal chosen from a class consisting of tungsten, molybdenum, mixtures of the two, and ferrous alloys containing at least 15% of any of the foregoing, hot coated with a bonded layer of aluminum containing substantially 5% to 15% beryllium, and substantially 5% to 15% silicon.

3. As a new article of manufacture, a refractory metal body protected from surface deterioration at elevated operating temperatures comprising a core constituted of a refractory metal selected from the group consisting of tungsten, molybdenum, alloys of tungsten and molybdenum, and alloys containing at least 15% of any of the foregoing with at least one of the metals iron, nickel, cobalt and chromium, and a protective layer on said core of aluminum containing substantially 5% to 15% beryllium.

4. As a new article of manufacture, a refractory metal body protected from surface deterioration at elevated operating temperatures comprising a core constituted of a refractory metal selected from the group consisting of tungsten, molybdenum, alloys of tungsten and molybdenum, and alloys containing at least 15% of any of the foregoing with at least one of the metals iron, nickel, cobalt and chromium, and a protective layer on said core of aluminum containing substantially 5% to 15% beryllium, and substantially 5% to 50% silicon.

5. The structure claimed in claim 3, with a thin interface layer of nickel between the body and the protective layer.

6. The structure claimed in claim 4, with a thin interface layer of nickel between the said body and the said protective layer.

7. A body formed from metal chosen from a class consisting of tungsten, molybdenum, mixtures of the two and ferrous alloys containing at least 15% of any of the foregoing, hot coated with a bonded layer of beryllium.

## References Cited in the file of this patent

## UNITED STATES PATENTS

|           |             |                |             |
|-----------|-------------|----------------|-------------|
| 1,155,317 | Mark        | Sept. 28, 1915 | 2,135,652   |
| 1,716,943 | Archer      | June 11, 1929  | 2,565,768   |
| 1,860,793 | Weiger      | May 31, 1932   | 2,588,421   |
| 1,879,748 | Horsfield   | Sept. 27, 1932 | 2,665,475   |
| 2,062,329 | Nock        | Dec. 1, 1936   | 5 2,682,101 |
| 2,096,924 | Schwarzkopf | Oct. 26, 1937  | 240,411     |
| 2,121,084 | Kruh        | June 21, 1938  | 723,418     |

|           |               |
|-----------|---------------|
| Whitfield | Nov. 8, 1938  |
| Gittings  | Aug. 28, 1951 |
| Shepard   | Mar. 11, 1952 |
| Campbell  | Jan. 12, 1954 |
| Whitfield | June 29, 1954 |

## FOREIGN PATENTS

|               |              |
|---------------|--------------|
| Great Britain | July 8, 1926 |
| France        | Apr. 8, 1932 |